

## UNITED STATES PATENT OFFICE

1,985,764

## COOKING UTENSIL

Albert L. Clapp, Danvers, Mass.

No Drawing. Original application March 12, 1926, Serial No. 94,329. Divided and this application February 21, 1929, Serial No. 341,849

4 Claims. (Cl. 53—6)

In my application Serial No. 94,329, filed March 12, 1926, of which the present case is a division, I have disclosed a composition of matter comprising fibrous material and setting or hardening compounds, wherein such compounds are present in such quantities as fully to saturate or permeate the fibrous material, and in which the fibrous material is present in closely interfelted condition, having preferably the closely interfelted conditions such as is produced by paper-making methods. Such a composition by the use of suitable setting or hardening compounds may possess certain desirable properties, such as being water-, grease- and fire-resistant, and being mouldable under certain conditions. This application is a division of my application hereinbefore identified, and relates to articles, and more particularly cooking utensils, made from the composition.

If asbestos be treated with sodium silicate, particularly in the presence of lime, a plastic compound results, which sets to a rigid, greaseproof and fireproof condition. The set composition, however, is of low strength and consequently is not suitable for formation into articles. I have found, however, that if asbestos fiber is employed together with cellulose fiber and then formed on a paper machine, a sheet of sufficient strength is produced, which when treated with sodium silicate may then be formed into various articles having certain desirable characteristics.

In accordance with the present invention, asbestos fiber and wood or other cellulosic fiber are intermixed by the usual beating operation, pulverulent lime being added and incorporated into the pulp while it is being beaten. The pulp is then sheeted on a paper-forming machine, and dried. The dry sheet is passed into a bath of sodium silicate and is permitted to become thoroughly saturated with the solution, whereupon the excess sodium silicate is expressed from the sheet and the sheet is allowed to stand or condition until it has been reduced to the proper temper or consistency for moulding into articles without tending to disintegrate. While in such temper, it may be bent and stamped into various articles without being cracked or broken, and in this respect behaves somewhat like ductile sheet metal, such as sheet tin, zinc, and the like. The article thus formed is finally dried, which may be facilitated by placing it in a warm, dry atmosphere, or by blowing warm, dry air thereupon, whereupon a permanent hardening or setting of the material takes place, resulting in a compara-

tively rigid material, which is greaseproof, fireproof and water-resistant.

While in temper, the material may be formed, for example, into baking utensils, such as cake pans, pie pans, and the like, by stamping blanks cut from the sheet material, which after setting are adapted for use as substitutes for utensils made from sheet metal. Such utensils retain their form under baking temperatures, and the flavor of the food is not deleteriously affected while being baked, since there are no malodors which arise from the utensil, even though carbonization of the cellulose fibers does take place. Even when subjected to the full blast of a Bunsen burner flame, the pan retains its form, although a decomposition and carbonization of the cellulosic fiber results, together with the formation of carbon dioxide. The utensils, moreover, while not perfectly waterproof, are sufficiently waterproof to resist disintegration by moisture or wet food; but after such utensils have been subjected to baking temperatures, they are quite waterproof.

Since such baking utensils may be produced economically, they may be used in place of the usual baking pans made of metal, and the baked goods be retained therein after baking, thus avoiding the necessity of the usual paper plates to which the pies or other baked materials are commonly transferred after baking. They thus serve a double use.

To produce sheet material suitable for formation into various articles, I may, for example, proceed as follows. Sixty parts of wood fiber and 40 parts of asbestos fiber are placed in the beater engine and sufficient water is added to ensure circulation. The fibers are thoroughly intermixed by beating for about twenty minutes, during which time about 10% to 15% lime, based on the dry weight of fiber, is added to the beater engine. The pulp is then run off and sheeted on a cylinder or a Fourdrinier machine, and the web formed is dried. The dried web or sheet is passed through a bath of sodium silicate, of about 20° Baumé, produced as by mixing equal parts by weight of a solution of sodium silicate (60° Baumé) and water, and is permitted to become saturated thoroughly therewith. The excess sodium silicate is removed from the sheet by passing it through squeeze rolls.

The sodium silicate acts upon the asbestos and appears to destroy the fibrous characteristic thereof, producing a plastic, more or less gummy composition throughout the sheet, which behaves in some respects like Portland cement, as it becomes set.

Immediately after passage through the sodium silicate bath, the sheet is weak and flabby, and does not successfully permit of article formation, but upon standing for a period it undergoes a change in temper and may be successfully subjected to forming operations. While in such condition, the sheet may, for example, be rolled up, or unrolled, and there is little, if any, tendency for successive convolutions to become united unless subjected to pressure. The sheet may be kept in temper when subjected to humid conditions, for some hours, after which a hardening of the material takes place even under conditions of high humidity.

While in temper, the sheet material may be stamped into such articles as baking pans, or formed into cans, boxes, tubes and other products. In such condition, the material also possesses the property of being "self-sealing," i. e., two layers of the material may be united without the use of an external binder or adhesive, by exerting sufficient pressure on the two layers and then allowing a hardening of the material to take place, which may be facilitated by subjecting it to warm, dry conditions. By this means, the layers are caused to unite, the hardening of the material effecting a permanent union between the layers. In forming such articles as boxes, cans and tubes from the material, this property is very advantageous, inasmuch as the joints or seams may be effected by the application of pressure on the abutting edge portions of properly cut blanks, and without employing any adhesives.

When the material has rigidified or set, it is greaseproof and oilproof, and consequently is admirably adapted for use in the formation of such articles as paint and oil containers, baking pans, and the like. Thus, for example, in baking cakes, the surface of the baking pan may be greased without danger of penetration through the utensil, thus permitting ready removal of the baked material.

If desired, the grease-resisting property of the container may be enhanced by applying a coating of glue or other greaseproofing material thereto. In addition, sizing or waterproofing agents, as in the form of insoluble soaps or wax, may also be applied, either alone or together with the greaseproofing agent, to the surface of the material. Such agents, however, are preferably not employed when the material is to be formed into articles which are to contact with foodstuffs, inasmuch as the taste of the food might be deleteriously affected.

Sheet material made as herein specified may be formed into thin sheets on a papermaking machine, having a thickness of as low as 5 to 6 points or thousandths of an inch, although for ordinary article formation the material is preferably formed to a thickness of about 7 to 8 points, or greater. For forming tubes or conduits, however, a sheet of considerable thickness may be produced and then wound, although a relatively thin sheet may be wound upon a mandrel and the successive convolutions be sufficiently pressed together to ensure a union therebetween and a substantially homogeneous tube produced, which, when permitted to harden, has all the successive convolutions permanently united.

In addition, the sheet material is very light, amounting to about 1/12 to 1/15 the weight of sheet tin of the corresponding caliper.

Articles of substantial thickness may also be

formed by winding or otherwise superposing several layers of the sheet material while in temper, and then uniting and moulding the layers into the desired articles under sufficient pressure to effect a permanent union therebetween. By this means, after the setting or hardening of the material has taken place, a dense, hard and "stony" material is produced.

While the incorporation of pulverulent lime into the stock prior to sheeting on a paper-forming machine may be dispensed with, yet I find it preferable to use lime. The lime also reacts with the sodium silicate to form a hardening compound, and acts to effect a better "conditioning" or control of the temper of the material for forming operation, aiding in producing a product possessing the required characteristics. When lime is not used in the furnish, however, the sheeted material after passage through the sodium silicate bath is more or less flabby and difficult to form without collapse and breakage of the sheet, even after tempering. The use of lime in addition ensures a better absorption and retention of the sodium silicate within the sheet, rather than permitting a surface absorption only; and also controls the rate of setting of the mixture of asbestos and sodium silicate; and imparts the physical characteristics desired in order to mould or stamp the sheet, and also certain of the desired characteristics in the sheet after hardening.

The use of cellulosic pulp, e. g., sulphite pulp or mechanical wood pulp, together with the asbestos fiber in forming the sheet, however, is indispensable. Not only does the cellulosic fiber impart strength and body to the web during paper-forming operation and production, but serves as an excellent absorbing medium to retain sufficient sodium silicate within the sheet to ensure characteristics desired in the finished product.

In certain instances, but with disadvantage, however, the use of asbestos in the furnish may be dispensed with and substituted by other hardening material. In such instance, the percentage of lime or other equivalent compound which reacts with sodium silicate to form a hardening compound and which is incorporated into the stock prior to sheeting on a paper machine or otherwise forming the fibers into an interfelted material, is raised to about 20% or more. In order to impart greater body to the material, especially when it is to be employed where its fireproof property is of prime importance, in addition to the lime, certain inorganic fillers, such as pulverulent kieselguhr and "cellite," may be incorporated into the pulp prior to its "formation."

While I have described a specific example of procedure which may be followed in producing a sheet suitable for a variety of uses, and certain articles of manufacture which may be produced therefrom, it should be obvious that this is by way of illustration only and that various modifications of procedure may be employed and that the material may be put to other use for which it may be found suitable. For instance, in the example given, I may employ 60 parts of asbestos fiber and 40 parts of cellulose fiber, or other proportions of asbestos and cellulose fiber. In general, however, I find it preferable to employ approximately equal parts of the two fibers. The proportion of lime used is also subject to variation, and while preferably employed in the proportions stated, may be somewhat increased or

decreased, and may, if desired, be replaced in part or entirely by other conditioning agents, e. g., certain pulverulent alkaline earth compounds, such as limestone, magnesium oxide, 5 magnesium carbonate, or certain other compounds, such as manganese dioxide.

Where the material which is capable of reacting with the sodium silicate to form a hardening compound is first incorporated into the fibrous material prior to "formation," and such fibrous material "formed" into interfeltd material, and then saturated with a solution of sodium silicate, the setting or hardening compound permeates or saturates the material as a continuous, coherent 10 body. Such a process cannot be considered to be equivalent in any sense to a process wherein both lime and sodium silicate are added to fibrous material prior to "formation," this latter process merely resulting in a filler being precipitated on the fibrous material in a pulverulent condition but without carrying the interfeltd fibrous material and permeating or saturating it, as is the condition in the present process. Nor is the material produced equivalent to the product 15 prepared by treating or immersing interfeltd fibrous material in a bath of hardening or setting compounds, as in a cement paste, and then permitting the material to rigidify.

It will be noted that according to the present invention, two agents which react together to form a hardening or setting compound are employed, and that this reaction is produced within the previously felted fibrous material, this being effected by incorporating one of these agents with the pulp prior to interfelting it, and then treating 20

the interfeltd material having the agent therein with the hardening or setting reagent.

Having thus described the nature of my invention and described a way of making and using the same, although without attempting to set forth all the forms in which it may be made or all the modes of its uses, what I claim is:

1. A cooking utensil formed from a normally inflammable absorptive material rendered resistant to heat at baking temperatures by impregnation with a fireproofing substance which will not exude at baking temperatures and coated on its inner surface with a water resistant material which will penetrate the body of the utensil at 10 baking temperatures. 15

2. A cooking utensil formed from a normally inflammable absorptive material rendered resistant to heat at baking temperatures by impregnation with a fireproofing substance which will not exude at baking temperatures and coated on its 20 inner surface with paraffine of relatively high melting point.

3. A cooking utensil of the character of a pie-plate, baking pan or the like, comprising a molded structure of interfeltd fibers containing, besides 25 cellulose film, at least about 40% asbestos as a component imparting heat-resistance thereto, said structure being impregnated with and stiffened by sodium silicate.

4. A cooking utensil of the character of a pie-plate, baking pan or the like, comprising a molded structure of interfeltd fibers containing both cellulose fiber and asbestos fiber, said structure being impregnated with and stiffened by sodium 30 silicate. 35

ALBERT L. CLAPP.